

May 6, 1952

H. A. REECE

2,595,295

WEDGE TESTING

Filed June 15, 1950



FIG. 2

FIG. 3



FIG. 7



FIG. 5

FIG. 6

INVENTOR.  
HERBERT A. REECE  
BY  
*William J. Leder*  
ATTORNEY.

## UNITED STATES PATENT OFFICE

2,595,295

## WEDGE TESTING

Herbert A. Reece, Cleveland Heights, Ohio

Application June 15, 1950, Serial No. 168,246

9 Claims. (Cl. 75—130)

1

This invention relates to wedge testing, but has reference more particularly to testing of iron used in manufacturing cast iron products.

In the production of iron for use in the manufacture of cast iron products, the degree or extent of graphitization or hardening is usually determined in the foundry through the use of chill test pieces or wedges.

In the wedge test, a casting about five inches long and of wedge-shaped cross-section is poured from the iron, this wedge-shaped casting having an acute angle at its apex, which angle, as well as the dimension of the back face of the wedge, may vary. After the wedge-shaped casting is poured and has been cooled, it is broken in two transversely so that the carbide balance may be observed on the broken surface of the casting at the line of demarcation between the metal of white appearance and the metal of gray appearance. The width measured across the broken surface of the wedge-shaped casting at the line of demarcation between the white portion of the wedge and the gray portion of the wedge is an indication of the section of casting which may be poured with the particular ladle of iron tested. As for instance, if the white portion of the wedge measures  $20/32$  then any casting of less than  $5/8$ " section will be white and unmachinable while any casting of more than  $3/4$ " section will be gray and machinable and a casting section between  $5/8$ " and  $3/4$ " will be mottled (composed of both white iron and gray iron).

The wedge test is said to have been originated by John Shaw, of England, about 1911, and is referred to in an article by O. Smalley on page 491 of volume 37 (1929) of the Transaction of the American Foundrymen's Association. The wedges or wedge-shaped castings are made in various sizes, the most beneficial angles, for general gray iron castings, being  $28^\circ$ ,  $26^\circ$  and  $16^\circ$ . The varying of the angle makes the wedge responsive to many sections to be cast, as for instance, when the combined properties of strength and machinability are sought, the  $28^\circ$  or the  $26^\circ$  wedge portion may be used. When the property sought is solely machinability, the  $16^\circ$  wedge portion may be used and when hardness and wear resistance is desired in the casting, the  $26^\circ$  wedge portions may be used for metal control test purposes.

One of the principal difficulties in the use of the wedge test has been the cost of the wedges. It is the usual practice to pour two wedges of different sizes and angularities, since if only a light wedge is poured, this wedge may prove to be all white and therefore unmeasurable, as when an improper amount of hardening agent or graphitizing agent has been used. In some cases, three wedges have to be poured.

The necessity of thus pouring two or more wedges causes a delay or delays in the pouring of

2

the ladle of iron, since the ladle man has to await approval of pouring, based on the tests. Thus, if the first wedge broken is unmeasurable, the iron control man must break a second wedge to determine the measurement of the white portion, in case a hardening agent is used, or the gray portion, in case a graphitizing agent is used, or the measurement between white and gray in case a combination of hardener and graphitizer is used.

The present invention has as its primary object improvements in the wedge test, which are designed to overcome the difficulties and disadvantages hereinabove described, and to facilitate a pouroff of the iron with a minimum of delay.

Another object of the invention is to provide improvements in the wedge test, which are designed to produce accurate, dependable, test results, effect a savings in the amount of iron used for the test, and reduce the cost of the tests from the viewpoint of labor and time required for the tests.

A further object of the invention is to provide a wedge test piece of novel contour and design.

A still further object of the invention is to provide an anvil of novel design for use in conjunction with such test piece.

Other objects and advantages of the invention will be apparent during the course of the following description.

In the accompanying drawing, forming a part of this specification, and in which like numerals are employed to designate like parts throughout the same,

35 Fig. 1 is a side elevational view of a typical test piece embodying the novel features of the invention;

Fig. 2 is a top plan view of the test piece;

Fig. 3 is a rear elevational view of the test side;

40 Fig. 4 is a cross-sectional view, taken on the line 4—4 of Fig. 1;

Fig. 5 is a cross-sectional view, taken on the line 5—5 of Fig. 1;

Fig. 6 is a cross-sectional view, taken on the line 6—6 of Fig. 1, and

Fig. 7 is a perspective view of an anvil embodying the invention, designed for use in conjunction with the test piece of Figs. 1 to 6.

A test piece, such as shown in Fig. 1 is made in a core or mold, such, for example, as a baked oil sand mold. For this purpose, a single pattern box may be used or a gang box may be used to make several test pieces at one time.

The test piece, it will be noted, comprises a flared head 1, a portion 2 immediately below the head, of uniform cross-section, which is desirable for heavy castings, a portion 3 below the portion 2, of uniform cross-section, which is desirable for medium castings, and a portion 4 below the portion 3, of uniform cross-section, which is desirable for light castings.

The back faces of the portions 2, 3 and 4 are coplanar with each other, but the knife-like edges of the respective portions, as shown in Fig. 1, are offset from each other, this offsetting resulting from the differences in the dimensions of the back faces and the differences in the angularities of the wedges.

Referring to Fig. 7 of the drawings, there is shown an anvil or block of iron having slots or passageways 5, 6 and 7, extending therethrough, slightly larger in cross-section than the portions 2, 3 and 4, respectively, of the test piece for easy insertion and withdrawal of the test wedge.

The portion of the test piece to be broken is slipped into its corresponding slot or passageway in the anvil to a depth equivalent to one-half of the length of that portion of the test piece, and is hit with a hammer, after which the desired reading or measurement is taken by observation of the fracture. By having the slots or passageways extending entirely through the anvil from front to rear, a punch may be used from the rear to eject the broken wedge section. The anvil should be firmly anchored in a suitable base.

If the broken section fails to give the desired information, it is a simple matter to easily and quickly insert one or both of the other portions of the test piece into the anvil or block, and obtain fractures for measurement of the degree of graphitization or hardening.

By thus pouring a single test piece with sections or portions of different angularities and dimensions corresponding to those considered most beneficial for the particular iron which is being produced, a saving in the amount of iron and number of cores used for the test is effected, as well as a reduction in the labor and time required for the tests, as a result of which delays are reduced to a minimum, and pouroff of the molten iron is greatly speeded. The test, moreover, produces accurate, dependable, results.

It is to be understood that the form of my invention, herewith shown and described, is to be taken as a preferred example of the same, and that various changes in the shape, size and arrangement of parts may be resorted to, without departing from the spirit of my invention or the scope of the subjoined claims.

Having thus described my invention, I claim:

1. The method of controlling the carbide balance in the production of castings from molten iron, which comprises pouring from the iron a single test specimen consisting of a plurality of standard wedges of different cross-sectional area and different angularity at the wedge edge, permitting the specimen to become solidified, severing the test specimen transversely of one of the wedges for observation of the carbide balance in said wedge, and similarly severing as many of the other wedges as necessary for observation of the carbide balance therein, if the first wedge fails to reveal the desired information, and adjusting the composition of the molten iron in accordance with the revelation of the specimen to obtain the desired properties in the castings.

2. The method, as defined in claim 1, in which the wedges are in end to end arrangement, with the back faces of all of the wedges coplanar.

3. The method, as defined in claim 2, in which the wedge edges of the wedges are out of alignment with each other.

4. The method, as defined in claim 3, in which the wedges are in vertical tier arrangement, each

wedge having a portion overhanging the wedge edge of the wedge immediately therebelow.

5. The method, as defined in claim 1, in which said adjustment comprises adjusting the degree of graphitization or hardening of the molten iron.

6. The method of controlling the carbide balance in the production of castings from molten iron, which comprises pouring from the iron a single test specimen consisting of a plurality of standard wedges of different cross-sectional area and different angularity at the wedge edge, permitting the specimen to become solidified, severing the test specimen transversely of at least one of the wedges for observation of the carbide balance in said wedge, and adjusting the composition of the molten iron in accordance with the revelation of the specimen to obtain the desired properties in the castings.

7. The method of controlling the carbide balance in the production of castings from molten iron, which comprises pouring from the iron a single test specimen of elongated form and of substantially triangular cross-sectional area varying from a minimum at the lower end of the specimen to a maximum at the upper end of the specimen, the specimen having a flat rear face and a wedge edge remote from said rear face, the angularity of said wedge edge varying from the lower end of the specimen to the upper end of the specimen, permitting the specimen to become solidified, severing the test specimen transversely at one point of its length for observation of the carbide balance at this point, and similarly severing the specimen transversely at as many other points of its length as necessary for observation of the carbide balance therein, if the observation at the first point fails to reveal the desired information, and adjusting the composition of the molten iron in accordance with the revelation of the specimen to obtain the desired properties in the castings.

8. The method, as defined in claim 7, in which said adjustment comprises adjusting the degree of graphitization or hardening of the molten iron.

9. The method of controlling the carbide balance in the production of castings from molten iron, which comprises pouring from the iron a single test specimen of elongated form and of substantially triangular cross-section from top to bottom thereof, with the cross-sectional area varying from a minimum at the lower end of the specimen to a maximum at the upper end of the specimen, the specimen having a flat rear face, and a wedge edge remote from said rear face, the angularity of said wedge edge varying from the lower end of the specimen to the upper end of the specimen, permitting the specimen to become solidified, severing the specimen transversely at at least one point of its length for observation of the carbide balance therein, and adjusting the composition of the molten iron in accordance with the revelation of the specimen to obtain the desired properties in the castings.

HERBERT A. REECE.

#### REFERENCES CITED

The following references are of record in the file of this patent:

#### UNITED STATES PATENTS

| Number    | Name    | Date           |
|-----------|---------|----------------|
| 2,359,044 | McBride | Sept. 26, 1944 |
| 2,371,654 | Smalley | Mar. 20, 1945  |
| 2,378,992 | Franks  | June 26, 1945  |